

# United States Patent

[11] 3,616,420

[72] Inventor **Trevor Broughton**  
Beaconsfield, England  
[21] Appl. No. **778,752**  
[22] Filed **Nov. 25, 1968**  
[45] Patented **Oct. 26, 1971**  
[73] Assignee **The British Aluminium Company Limited**  
London, England

[56]

## References Cited

### UNITED STATES PATENTS

|           |         |                   |        |
|-----------|---------|-------------------|--------|
| 3,227,644 | 1/1966  | Rutemiller.....   | 75/146 |
| 3,281,239 | 10/1966 | Reding et al..... | 75/147 |
| 3,343,948 | 9/1967  | Raclot.....       | 75/147 |

Primary Examiner—Richard O. Dean

Attorney—Peck & Peck

[54] **ALUMINUM BASE ALLOYS AND ANODES**  
16 Claims, No Drawings

[52] U.S. Cl. .... **204/197,**  
75/140, 75/141, 75/146, 204/148, 204/293  
[51] Int. Cl. .... **C23f 13/00**  
[50] Field of Search.... **75/146,**  
147, 148, 140, 141; 148/32, 32.5; 204/148, 197,  
293

**ABSTRACT:** Aluminum base alloys which are suitable for use in the as cast state as galvanic anodes, the alloys comprising 1-15% zinc, 0.005-0.1% indium and 0.4-10% magnesium, the balance being aluminum of at least 99.8 percent purity with inconsequential impurities. The alloy may optionally include some tin, for example in the range of 0.1-0.5 percent, some gallium in the range of from 0.005 to 0.017 percent and a grain refiner such as titanium and zirconium.

## ALUMINUM BASE ALLOYS AND ANODES

### BACKGROUND OF THE INVENTION

The requirements for galvanic anodes are a high operating potential and a high efficiency measured as electrical output per unit mass of metal consumed.

Many conventional alloys used for forming anodes, for example aluminum-zinc-tin alloys in production at the present time require a heat treatment after being cast before they are suitable for use. There are considerable economic and technical advantages in being able to produce high capacity sacrificial anodes which will operate satisfactorily in the as-cast condition without the necessity for formal heat treatment.

### BRIEF SUMMARY OF THE INVENTION

We have found that the incorporation of magnesium in an aluminum-zinc-indium alloy in the correct proportion provides a satisfactory as-cast product.

Accordingly the invention provides in one aspect an aluminum base alloy comprising 1-15 percent zinc, 0.005-0.1 percent indium and 0.4-10 percent magnesium, the balance being aluminum of at least 99.8 percent purity with inconsequential impurities.

The proportion as impurities of silicon and iron should each preferably be below 0.2 percent. Preferably the zinc content is between 2 and 10 percent and with advantage between 2.5 and 8 percent. Preferably the indium content is between 0.01-0.05 percent and with advantage between 0.03 and 0.04 percent. Preferably the magnesium content is between 0.4 and 1 percent and with advantage is between 0.6 and 0.8 percent particularly where restrictions to incendive sparkling apply. The alloy may also include some tin, for example in the range 0.1 percent to 0.5 percent.

It is preferable to include some gallium in the range 0.005 to 0.017 percent and preferably for example 0.01 percent.

In this specification all percentages are by weight.

It is further preferred to include a grain refiner of any suitable form (for example titanium and zirconium) to improve the cast product.

In another aspect the invention provides an anode in the as-cast state made from an alloy as set out above.

The melt was then thoroughly stirred with the temperature controlled between 710°-730°C.

Casting was then carried out into dies held at 100°-250°C.

Half inch sections were cut from 1 inch-diameter test bars 5 of the material to be tested and electrical connections made through a threaded length of  $\frac{1}{4}$ -inch diameter aluminum rod screwed into the upper machine surface of the specimen. Both machined surfaces were marked off using a stopping off medium and the weighed samples were then mounted concentrically in 9-inch diameter 12-inch high, shot-blasted mild steel drums containing about 11 liters of natural sea water. Gentle agitation by stirring was used during the test and the electrolyte in the tank was changed regularly. The tests were carried out at laboratory temperatures.

15 The current supplied by the dissolving anode after being connected to the steel drum was restricted to an anode current density of 10 ma./in.<sup>2</sup> by means of a variable resistor in the external circuit. The potential drop across a further accurately calibrated resistor (also in the external circuit) was used to monitor the current flow and these values were recorded automatically every four hours during test. The total current supplied by the anode section could therefore be calculated.

20 The period of testing varied from 40-60 days by which time about 50 percent of the specimen had been consumed. After removing from the test environment specimens were cleaned in 1:1 nitric acid (to remove adherent corrosion product,) and were then reweighed after drying.

25 The theoretical output for the particular weight loss of the 30 specimen was calculated using an electrochemical equivalent for the particular alloy on test (i.e. allowance made for the zinc content of the alloy) and the efficiency calculated as the percentage of the theoretical output actually supplied by the anode during testing.

35 Potentials were measured at regular intervals throughout the test using a saturated calomel electrode in contact with the dissolving aluminum anode or on the outside of any adherent corrosion present on the specimen surface. The value of potential quoted is that measured on the final day of the test.

40 Examples of specifications of and properties of anodes made from alloys in accordance with the invention are shown in table 1.

TABLE I

| Alloy identification | Base purity | Composition |      |        |       |         | Efficiency at 10 ma./in. <sup>2</sup> percent | Operating potential at 10 ma./in. <sup>2</sup> (-mv. versus saturated calomel electrode) |
|----------------------|-------------|-------------|------|--------|-------|---------|-----------------------------------------------|------------------------------------------------------------------------------------------|
|                      |             | Magnesium   | Zinc | Indium | Tin   | Gallium |                                               |                                                                                          |
| A                    | 99.8        | 0.60        | 3.52 | 0.030  | ----- | 0.007   | 86                                            | 1,110                                                                                    |
| B                    | 99.8        | 0.78        | 3.54 | 0.030  | ----- | 0.009   | 92                                            | 1,120                                                                                    |
| C                    | 99.8        | 0.64        | 5.01 | 0.035  | ----- | 0.010   | 90                                            | 1,100                                                                                    |
| D                    | 99.8        | 0.62        | 2.51 | 0.030  | ----- | 0.008   | 91                                            | 1,100                                                                                    |
| E                    | 99.8        | 0.60        | 3.55 | 0.025  | ----- | 0.010   | 91                                            | 1,100                                                                                    |
| F                    | 99.8        | 0.62        | 3.54 | 0.050  | ----- | 0.009   | 89                                            | 1,110                                                                                    |
| G                    | 99.8        | 0.67        | 3.51 | 0.03   | 0.09  | 0.008   | 85                                            | 1,100                                                                                    |
| H                    | 99.8        | 0.99        | 3.95 | 0.048  | 0.09  | 0.010   | 81                                            | 1,060                                                                                    |
| I                    | 99.8        | 0.36        | 3.57 | 0.035  | ----- | 0.010   | 85                                            | 1,000                                                                                    |

### DESCRIPTION OF THE PREFERRED EMBODIMENTS

Some aluminum base anodes were made up and tested by way of example as follows:

60 Aluminum was melted and raised to a temperature of 710° C. Zinc, indium, (and in some cases tin) were added as required and this operation was followed by degassing. Magnesium was then added as required and to minimize oxidation effects additions were made under a layer of Coverall 33F.

It will be noticed that in the case of composition I where the magnesium content is below 0.4 percent the operating potential fell to -1,000 mv. and the resulting anode was less satisfactory than those of higher magnesium contents.

Further examples of specifications of and properties of anodes made from alloys in accordance with the invention are shown in table II. In these examples, the copper content was in each case found to be less than 0.005 percent and the silicon and iron contents are shown.

TABLE II

| Alloy designation | Percent composition <sup>1</sup> |      |      |      |       | Efficiency at 10 ma./in. <sup>2</sup> percent | Potential at 10 ma./in. <sup>2</sup> -mv. (versus saturated calomel electrode) |
|-------------------|----------------------------------|------|------|------|-------|-----------------------------------------------|--------------------------------------------------------------------------------|
|                   | Mg                               | Si   | Fe   | Zn   | In    |                                               |                                                                                |
| J                 | 0.69                             | 0.10 | 0.06 | 3.54 | 0.032 | 0.012                                         | 96                                                                             |
| K                 | 0.70                             | 0.04 | 0.10 | 3.55 | 0.033 | 0.012                                         | 86                                                                             |
| L                 | 0.70                             | 0.04 | 0.03 | 3.52 | 0.030 | 0.011                                         | 93                                                                             |
| M                 | 0.72                             | 0.17 | 0.08 | 7.63 | 0.03  | 0.012                                         | 88                                                                             |
| N                 | 0.68                             | 0.04 | 0.04 | 3.58 | 0.03  | 0.011                                         | 87                                                                             |
| O                 | 0.71                             | 0.08 | 0.06 | 4.59 | 0.034 | 0.012                                         | 84                                                                             |

<sup>1</sup> Balance Al of 99.8% purity.

The applicants have investigated the effect of variations in casting techniques on the electrochemical properties of alloys according to the invention. These investigations involved variations in the liquid metal temperature, variations in the mould temperature and variations in the cooling technique. Three cooling techniques were tried, one of these identified as the standard procedure involved casting the metal into a mold and, when it had become sufficiently solidified, removing it from the mold and allowing it to cool, the second technique identified as "water quench-cold water" involved casting the metal into a mold and, when it had become sufficiently solidified, removing it from the mold and quenching it in cold water, and the third technique identified as "very slow cool in molds" involved casting the metal into a mold and allowing it to cool in the mold to ambient temperature. This latter technique gave a retarded rate of cooling and a superior result as can be seen from table III below. The alloy used for the investigation of which the results are given in table III was an alloy containing 0.68 percent magnesium, 4.01 percent zinc, 0.038 percent indium, 0.012 percent gallium, 0.12 percent silicon, 0.07 percent iron and less than 0.005 percent copper.

TABLE III

| Casting conditions       |                           |                               | Potential at 10 ma./in. <sup>2</sup> —mv. (versus saturated calomel electrode) |                                           |
|--------------------------|---------------------------|-------------------------------|--------------------------------------------------------------------------------|-------------------------------------------|
| Liquid metal temp. (°C.) | Average mould temp. (°C.) | Additional treatments         | Efficiency at 10 ma./in. <sup>2</sup> percent                                  | —mv. (versus saturated calomel electrode) |
| 720                      | 200                       | Standard procedure.....       | 76                                                                             | 1,100                                     |
| 720                      | 260                       | Water quench cold water.....  | 74                                                                             | 1,095                                     |
| 720                      | 360                       | Standard procedure.....       | 73                                                                             | 1,100                                     |
| 800                      | 300                       | do.....                       | 79                                                                             | 1,115                                     |
| 720                      | 260                       | Very slow cool in moulds..... | 93                                                                             | 1,120                                     |

The addition of grain refining elements such as Zirconium and titanium to alloys according to the invention was investigated and the results are shown in table IV below. These results indicate that beneficial results are obtained with the addition of a grain refining element, preferably titanium in the range of from 0.005 to 0.07 percent and more specifically in the range from 0.01 to 0.04 percent. In each of the alloys shown in table IV the copper content was less than 0.01 percent.

TABLE IV

| Anode identification | Percent composition <sup>1</sup> |      |      |       |       |      | Efficiency at 10 ma./in. <sup>2</sup> (versus saturated calomel electrode) | Potential at 10 ma./in. <sup>2</sup> —mv. |
|----------------------|----------------------------------|------|------|-------|-------|------|----------------------------------------------------------------------------|-------------------------------------------|
|                      | Mg                               | Si   | Fe   | In    | Ga    | Zn   |                                                                            |                                           |
| G1.....              | 0.74                             | 0.08 | 0.06 | 0.031 | 0.01  | 3.75 | <.01                                                                       | 80                                        |
| G2.....              | 0.71                             | 0.09 | 0.06 | 0.030 | 0.013 | 3.82 | <.005                                                                      | 87                                        |
| G3.....              | 0.69                             | 0.09 | 0.06 | 0.034 | 0.01  | 3.79 | <.01                                                                       | 85                                        |
| G4.....              | 0.68                             | 0.08 | 0.07 | 0.036 | 0.01  | 3.79 | 0.02                                                                       | 94                                        |
| G5.....              | 0.73                             | 0.08 | 0.06 | 0.034 | 0.012 | 3.81 | 0.015                                                                      | 85                                        |
| G6.....              | 0.63                             | 0.07 | 0.06 | 0.037 | 0.01  | 3.75 | 0.02                                                                       | 83                                        |
| G7.....              | 0.69                             | 0.07 | 0.06 | 0.034 | 0.012 | 3.86 | 0.020                                                                      | 93                                        |
| G8.....              | 0.66                             | 0.07 | 0.07 | 0.035 | 0.01  | 3.81 | 0.02                                                                       | 81                                        |
| G9.....              | 0.70                             | 0.08 | 0.07 | 0.035 | 0.013 | 3.80 | 0.02                                                                       | 91                                        |
| G10.....             | 0.64                             | 0.08 | 0.08 | 0.037 | 0.01  | 3.81 | 0.02                                                                       | 95                                        |

<sup>1</sup> Balance Al of 99.8% purity.

I claim:

1. An aluminum base alloy for use as a sacrificial anode material consisting essentially of 1-15 percent zinc, 0.005-0.1 percent indium, 0.4-10 percent magnesium, 0-0.5 percent tin and 0-0.017 percent gallium the balance being aluminum of at least 99.8 percent purity with 99.8 impurities.

65

percent indium, 0.4-10 percent magnesium, 0-0.5 percent tin and 0-0.017 percent gallium, the balance being aluminum of at least 99.8 percent purity with inconsequential impurities, said anode having been cast in a mold and allowed to cool therein to ambient temperature.

\* \* \* \* \*